



US012351951B2

(12) **United States Patent**  
Morgis et al.

(10) **Patent No.:** US 12,351,951 B2  
(45) **Date of Patent:** \*Jul. 8, 2025

(54) **WEBBING FOR FALL PROTECTION DEVICE**

(71) Applicant: **OTEX Specialty Narrow Fabrics, Inc.**, Bernardsville, NJ (US)

(72) Inventors: **Mark M. Morgis**, Mountain Top, PA (US); **Kevin W. Raup**, Milton, PA (US)

(73) Assignee: **OTEX Specialty Narrow Fabrics, Inc.**, Bernardsville, NJ (US)

(\*) Notice: Subject to any disclaimer, the term of this patent is extended or adjusted under 35 U.S.C. 154(b) by 0 days.

This patent is subject to a terminal disclaimer.

(21) Appl. No.: **18/401,056**

(22) Filed: **Dec. 29, 2023**

(65) **Prior Publication Data**

US 2024/0133085 A1 Apr. 25, 2024

**Related U.S. Application Data**

(63) Continuation-in-part of application No. 16/427,717, filed on May 31, 2019, now Pat. No. 11,872,419.

(60) Provisional application No. 62/679,127, filed on Jun. 1, 2018.

(51) **Int. Cl.**

**D03D 1/00** (2006.01)

**D03D 11/00** (2006.01)

**D03D 15/47** (2021.01)

**D03D 13/00** (2006.01)

(52) **U.S. Cl.**

CPC ..... **D03D 1/0005** (2013.01); **D03D 11/00** (2013.01); **D03D 15/47** (2021.01)

(58) **Field of Classification Search**

CPC ..... D03D 1/0005; D03D 11/00; D03D 15/47; D03D 15/283; D03D 15/573; D10B 2321/0211

See application file for complete search history.

(56) **References Cited**

**U.S. PATENT DOCUMENTS**

- |                |                            |                        |
|----------------|----------------------------|------------------------|
| 1,734,165 A *  | 11/1929 Willard .....      | D03D 1/00<br>D11/221   |
| 4,856,837 A *  | 8/1989 Hammersla, Jr. .... | B66C 1/18<br>139/411   |
| 5,677,056 A *  | 10/1997 Golz .....         | D03D 15/292<br>428/192 |
| 6,840,066 B2 * | 1/2005 Dickerson .....     | D04B 21/18<br>66/195   |
| 7,815,013 B2 * | 10/2010 Griffith .....     | A62B 35/04<br>182/18   |
| 7,866,245 B2 * | 1/2011 Kempf .....         | D07B 5/06<br>87/8      |
| 7,870,934 B2 * | 1/2011 Ecker .....         | A62B 1/08<br>182/234   |
| 8,356,691 B2 * | 1/2013 Griffith .....      | A62B 35/04<br>182/18   |

(Continued)

*Primary Examiner* — Robert H Muromoto, Jr.

(74) *Attorney, Agent, or Firm* — Lowenstein Sandler LLP

(57) **ABSTRACT**

A webbing for use in a fall protection device, such as a self-retracting lifeline having leading edge capabilities, is provided having a double cloth construction with the exterior of the webbing constructed of woven, ultra-high molecular weight polyethylene yarns and having stuffer yarns positioned in the interior of the fabric, wherein the stuffer yarns are made of high-tenacity fibers, such as aramid fibers.

**22 Claims, 2 Drawing Sheets**



(56)

**References Cited**

U.S. PATENT DOCUMENTS

- 8,701,716 B2 \* 4/2014 Kashihara ..... D03D 15/283  
139/384 R  
9,199,103 B2 \* 12/2015 Hetrich ..... A62B 1/10  
9,238,156 B2 \* 1/2016 Apel ..... A62B 35/0075  
9,719,196 B2 \* 8/2017 Salama ..... D03D 1/0052  
11,390,969 B1 \* 7/2022 Aerts ..... D03D 1/007  
11,872,419 B1 \* 1/2024 Morgis ..... D03D 1/0005  
2002/0124904 A1 \* 9/2002 Howland ..... B32B 5/26  
139/420 R  
2006/0027277 A1 \* 2/2006 Jennings ..... A62B 35/04  
139/408  
2008/0179136 A1 \* 7/2008 Griffith ..... A62B 35/04  
182/5  
2010/0101833 A1 \* 4/2010 Zachariades ..... B32B 5/02  
174/136  
2012/0205478 A1 \* 8/2012 Balquist ..... A62B 35/04  
242/380  
2014/0113519 A1 \* 4/2014 Golz ..... D02G 3/12  
57/235  
2015/0013079 A1 \* 1/2015 Golz ..... A62B 35/0075  
8/638  
2016/0220857 A1 \* 8/2016 Rappoport ..... A62B 35/0075

\* cited by examiner





*FIG. -2-*



*FIG. -3-*

## WEBBING FOR FALL PROTECTION DEVICE

### CROSS REFERENCE TO RELATED APPLICATIONS

This application is a Continuation-In-Part of and claims priority to U.S. patent application Ser. No. 16/427,717 filed on May 31, 2019, which claims priority to U.S. Provisional Patent Application No. 62/679,127 filed on Jun. 1, 2018, the entire contents of which is incorporated herein by reference.

### TECHNICAL FIELD

This invention relates to narrow textile fabrics in the form of webbing for use in a fall protection device, in particular, for leading edge applications.

### BACKGROUND

A fall protection device is a safety equipment used to prevent or minimize injuries from falls, especially in workplaces where employees work at heights. These devices are critical in industries like construction, roofing, telecommunications, window cleaning, and any other field where workers are exposed to the risk of falling from elevated positions. The types of fall protection devices can be categorized into several main groups. For example, a personal fall arrest system (PFAS) is designed to safely stop a person who is falling. A typical PFAS includes a full-body harness that distributes the force of the fall across the body, minimizing the risk of injury, an anchorage point or a secure point to which the harness is attached, and a connector, which may include includes lanyards, lifelines, and deceleration devices that connect the harness to the anchorage. Some connectors include mechanisms to absorb energy and reduce the force of the stop during a fall.

Other types include guardrail system, which are barriers erected along the edges of elevated work areas to prevent workers from falling. Guardrails are a form of passive fall protection as they do not require the worker to wear or do anything. Safety net systems can be placed below a high work area to catch falling workers and objects, reducing the risk of serious injury. Positioning device systems allow a worker to be supported on an elevated vertical surface, such as a wall or column, and work hands-free while leaning. They are not designed to stop a fall but to prevent one from occurring. Fall restraint systems include components like harnesses and lanyards, but they are set up to prevent the worker from reaching a point where they could fall. Retractable lifelines and lanyards allow some movement but lock quickly in the event of a fall, much like a seatbelt in a car.

The selection of a fall protection device depends on several factors, including the nature of the work, the work environment, and the height at which the work is being performed. In many regions, the use of appropriate fall protection equipment is mandated by occupational health and safety regulations for certain types of work. Regular training, maintenance, and inspection of fall protection equipment are also crucial to ensure the safety and effectiveness of these devices.

### SUMMARY

A webbing is provided having a double cloth woven construction enveloping a plurality of stuffer yarns. The webbing has two exterior sides and two edges. Each of the

sides is comprised of a plurality of warp yarns, also referred to as ends, interlaced crosswise multiple times along the length of the webbing with a weft yarn, also referred to as a filling yarn. Each insertion of the weft yarn through the warp yarns is referred to as a pick. The warp yarns are multifilament yarns comprised of ultra-high molecular weight polyethylene fibers. The weft yarn is a multifilament yarn comprised of high-tenacity fibers, which may be ultra-high molecular weight polyethylene or a different high-tenacity fiber. The warp and weft yarns may be interlaced to create a plain, twill or satin weave, or a combination thereof.

The first side and second side are joined together by binder yarns extending between the first side and the second side of the webbing, thereby joining the sides together. By way of example, the double construction may be self-stitched, center stitched, or stitched by yarn interchange. The binder may be a multifilament yarn comprised of high-tenacity fibers.

A plurality of stuffer yarns are sandwiched between the first side and the second side of the double cloth and extend in the warp direction. The stuffer yarns are multifilament yarns comprised of high-tenacity fibers, which provide strength and resilience to the webbing. The stuffer yarns are held in place by the binder yarns, and in certain embodiments, by a continuous weft yarn encircling the first side and second side of the double cloth in a spiral, thereby joining their edges together. A catch cord may be employed along the edges of the webbing to lock the weft yarns in place and secure the stuffer yarns within the interior of the webbing.

A feature of the present invention is the concentration of the warp yarns at the exterior or face of each side of the webbing, that is, the warp yarns are predominantly exposed at the face of each side of the webbing, relative to the weft yarn. Accordingly, the ultra-high molecular weight polyethylene warp yarns, which have superior abrasion resistance and cut resistance, are exposed to an edge in a fall protection application. Furthermore, in the case of a fall, the webbing will be dragged along an edge, and it is believed to be advantageous for the yarns running lengthwise in the webbing, that is, the warp yarns, to engage the leading edge, rather than the weft yarn, to minimize snagging.

The objectives of the invention may be accomplished by one or more of the following constructions, or combinations thereof. The warp yarns may be provided in significantly higher concentration than the weft yarn. By way of example, the ratio of the ends per inch of warp yarns comprised of ultra-high molecular weight polyethylene to the picks per inch in the woven sides of the webbing may be 2:1 or greater, particularly, 3:1 or greater, more particularly 4:1 or greater. A single weft yarn may be employed, whereby the weft yarn is interlaced with the warp yarns in the first side of the webbing, next the weft yarn encircles a first edge of the webbing and is interlaced with the warp yarns in the second side of the webbing, and then the weft yarn encircles the second edge of the webbing and is again interlaced with the warp yarns in the first side of the webbing at a farther distance along the length of the webbing, thereby creating a continuous spiral. It can be understood that by controlling the tension of the weft yarn, the warp yarns are drawn together, forcing the exposure of the warp yarns on the face of each side of the webbing. An additional technique for improving the performance of the webbing in leading edge, fall protection applications is to minimize the picks per inch of the weft yarn to 24 ppi or less, in particular, from 6 to 18 ppi, more particularly, from 8 to 16 ppi, per side.

The webbing of the present invention has application in fall protection devices, especially due to the combination of

the webbing's abrasion and cut resistance, high tensile strength, flexibility and compact volume. The webbing may also be used in other applications where a high tensile strength webbing is desirable, such as towing, crane/load-bearing slings, climbing, load securing, passenger restraint in vehicles, military apparel, furniture, aerospace, first responder equipment, medical equipment, tactical gear and the like.

#### BRIEF DESCRIPTION OF THE DRAWINGS

FIG. 1 is a perspective view of the webbing with a  $\frac{1}{2}$  twist to show both sides.

FIG. 2 is a side view of the webbing showing the catch cord stitched into the side of the webbing.

FIG. 3 is a side view of the webbing showing an indicator yarn stitched into the side of the webbing.

The drawings are provided to illustrate the arrangement of the various yarns that make up the construction of the webbing of the present invention but are not intended to show the precise number of yarns.

#### DETAILED DESCRIPTION

Fall protection systems typically incorporate (i) a harness worn by a worker; (ii) a self-retracting lifeline and/or lanyard; and (iii) an anchor connected to the free end of the lifeline. If a worker falls, a locking mechanism in the housing prevents the pay out of the lifeline, thereby arresting the fall. A leading edge application is a working surface with a sharp or abrasive edge, such as a steel girder or concrete decking, which places additional stress on the lifeline, should a worker fall.

Various fall protection systems have been developed, which incorporate a textile made of high modulus synthetic fibers as the lifeline. The threads forming the edge of the webbing are characterized by outer edge threads and inner edge threads. The outer edge threads and inner edge threads are provided in contrasting colors. When the outer edge threads are worn, the inner edge threads are exposed, thereby indicating that the lifeline may need to be replaced.

Despite the developments in the field of fall protection, there remains a need for a lifeline for use in a fall protection system that is abrasion and cut resistant, high strength, able to absorb the shock of a person falling, flexible, lightweight, and compact.

Without limiting the scope of the invention, the preferred embodiments and features are hereinafter set forth. All of the United States patents and published patent applications cited in the specification are hereby incorporated by reference. Unless otherwise indicated, concentrations are by weight and molecular weight is based on weight average molecular weight. The term "polymer" as used in the present application denotes a material having a weight average molecular weight ( $M_w$ ) of at least 5,000. The term "copolymer" is used in its broad sense to include polymers containing two or more different monomer units, such as terpolymers, and unless otherwise indicated, includes random, block, statistical copolymers. The term "yarn" includes (i) monofilament; (ii) a plurality of continuous filaments laid together, with or without twist; and (iii) staple fibers twisted together. The term "multifilament yarn" is used to identify a yarn having a plurality of continuous filaments laid together, with or without twist. Yarns may be in the form of individual strands, multiple strands plied together, or multiple plied strands twisted together to form cord.

Referring to FIG. 1, webbing 1 is a double cloth construction. Webbing 1 has side 2 with warp yarns 3 and weft yarns 4, woven together. Webbing 1 is shown with a  $\frac{1}{2}$  twist in FIG. 1 to illustrate side 5, opposite from side 2. In the embodiment shown, weft yarn 4 from side 2 wraps around edge 8 of side 2 and edge 9 of side 5, before being inserted through warp yarns 6 of side 5. Next, weft yarn 4 emerges from edge 10 of side 5 and wraps around edge 11 of side 2. Thus, weft yarn 4 continuously wraps webbing 1 in a spiral to join the edges of side 2 and side 5 together.

It can be understood that instead of continuously wrapping weft yarns 4 around edges 8-11, weft yarn 4 may be interlaced with warp yarns 3 of side 2 and weft yarns 7 may be interlaced with warp yarns 6 of side 5, and for example, locked in place by a catch cord. Accordingly, as used herein, the term "weft yarn" refers to either a set of yarns that interlace with the warp yarns of a single side, or a single yarn that interlaces with the warp yarns on one side of the webbing and is wrapped around the edges to interlace with the warp yarns on a second side of the webbing, etc.

Warp yarns 3 and warp yarns 6 are multifilament yarns comprised of ultra-high molecular weight polyethylene (UHMWPE) fibers, also known as high-modulus polyethylene (HMPE) fibers. The UHMWPE may have a molecular weight of 3 million or greater, and is marketed under the trademarks Dyneema® and Spectra®. By way of example, the warp yarns may range in denier from 1200d to 2000d, with a filament count of from 500 to 1500. In the example illustrated in FIG. 1, all of warp yarns 3 and 6 may be comprised of UHMWPE. It can be understood that the invention may be practiced with a plurality of the warp yarns being comprised of UHMWPE and other warp yarns being comprised of a different material. In certain embodiments, 50% by weight of the warp yarns are UHMWPE, in particular 66% by weight of the warp yarns are UHMWPE, and more particularly, 75% by weight of the warp yarns forming woven sides 2 and 5 are UHMWPE.

Weft yarns 4 (and 7 when applicable) may be comprised of multifilament, ultra-high molecular weight polyethylene fibers. Alternatively, weft yarns 4 may be comprised of high-tenacity fibers other than UHMWPE, for example, a multifilament, high-tenacity yarn.

The relative amount of warp yarns comprised of UHMWPE to weft yarns in each of the woven sides of the webbing may be expressed as a weight ratio. Accordingly, the weight of the warp yarns comprised of UHMWPE to the weight of weft yarns may be 2:1 or greater, in particular 3:1 or greater or even 3.5:1 or greater.

Side 2 and side 5 are joined together by binder yarns 12, extending between the two sides of webbing 1, thereby joining the two sides together, as shown in FIG. 1. By way of example, the double construction may be self-stitched, center stitched, or stitched by yarn interchange. Binder yarns 12 may be comprised of multifilament, ultra-high molecular weight polyethylene fiber, or binder yarns 12 may be comprised of yarns of high-tenacity fibers other than UHMWPE.

Side 2 and side 5 may be a plain, twill or satin weave. For example, face 13 of side 2 may be a 1x1 or 2x2 plain weave or a warp face twill weave, such as a 2/1, 3/1 or 4/1 twill weave. Face 14 of side 5 may be the same weave as side 2 or different. By way of example, the weave construction of each of sides 2 and 5 may be the same or different and range from 25 to 125 ends per inch and from 5 to 25 picks per inch, in particular from 40 to 100 ends per inch and from 6 to 18 picks per inch. In order to maximize the benefits of the UHMWPE warp yarns, especially in fall protection applications, side 2 and side 5 may be constructed to increase the

exposure of warp yarns 3 and warp yarns 6, respectively, relative to the weft yarns. In order to increase the number of warp yarns woven into each side of webbing 1, the warp yarns may be woven in pairs, or as plies of two or more yarns, or as cords of two or more plies.

Stuffer yarns 15 are positioned between side 2 and side 5 of webbing 1. Stuffer yarns 15 are multifilament yarns comprised of high-tenacity fibers. The term "high-tenacity" fibers is intended to include UHMWPE fibers, aramid fibers, such as para-aramid, for example Kevlar®, liquid crystal copolyester fibers, such as aromatic polyesters, for example Vectran®, poly(p-phenylene-2,6-benzobisoxazole), such as Zylon®, and other fibers having a tensile strength of 2.0 GPa or greater, in particular 2.5 GPa or greater, more particularly 3.0 GPa or greater, as well as combinations thereof. In one embodiment of the invention, stuffer yarns 15 comprise a high-tenacity fiber other than UHMWPE, in particular, a para-aramid fiber, such as Kevlar®.

Stuffer yarns 15 may range in denier from 800d to 2000d, with a filament count of from 500 to 1500. The ends per inch of stuffer yarns may range from 100 to 250. In one embodiment of the invention, the stuffer yarns are provided as a cord, that is, the stuffer yarns are plied together and the plied yarns are twisted into a cord, to improve strength and stability and to facilitate weaving. By way of example, the stuffer yarns may be used as 3x4 cords, that is, three single yarns are plied together to create a 3-ply yarn and four 3-ply yarns are twisted together to create a cord. By way of further example, 10 to 20 3x4 cords, representing 120 to 240 single yarns ends may be used.

The ratio of the combined weight of side 2 and side 5 to the weight of stuffer yarns 15 may range from 1:3 to 3:1, in particular, from 1:2 to 2:1, and more particularly from 1:1.5 to 1.5:1.

Webbing made according to teachings herein may have a tensile strength of 6,000 lbs. or greater per one inch width of webbing, as measured by ASTM D6775-13(2017).

Referring to FIG. 2, edges 8 and 9 and edges 10 and 11 may be provided with catch cord 16 and catch cord 17, respectively, to prevent webbing 1 from unraveling. Examples of the use of a catch cord may be found in U.S. Pat. No. 5,677,056.

Other fibers or yarns may be incorporated in webbing 1 for identification or to detect wear, as is known in the art, and illustrated by indicator yarn 18 in FIG. 3.

#### Example 1

A double cloth, plain weave webbing was produced on a needle loom. Each side of the webbing was constructed of 48 ends of 1600d, 1000 filament ultra-high molecular weight polyethylene yarns and 24 ends of 1000d, 192 filament polyester yarns along the edges of the webbing, and 12±2 ppi of 1600d, 1000 filament ultra-high molecular weight polyethylene yarns. The stuffer yarns were 1500d, 3x4 Kevlar® cord, and 14 cords (168 yarns) were positioned between the front and back sides of the webbing. Binder yarns of 1600d, 1000 filament ultra-high molecular weight polyethylene yarn binder were woven between the front and back to secure the sides together. A polyester catch cord (1000d/192/1.5z) was used to bind the edges of the webbing.

The webbing had a width of approximately 1.0 inches, a thickness of approximately 0.14 inches and a weight of approximately 58 g/linear yard. The tensile strength of the webbing was approximately 8,000 lbs.

#### Self-Retracting Lifeline

The webbing of the present invention is particularly useful as the lifeline component in a self-retracting lifeline.

Typically, a self-retracting lifeline includes a housing having a rotatable drum mounted on a shaft within the housing. The lifeline is wound around the drum. A snap hook at the free end of the lifeline is anchored to a stationary object, when a worker is operating at a potentially dangerous height. When the lifeline is paid out slowly, a spring mechanism within the housing maintains tension on the lifeline, to remove slack. If, however, the worker falls, a locking engages to prevent the lifeline from paying out, thereby arresting the fall. The locking mechanism may also incorporate a braking assembly, to prevent injury caused by an abrupt stop of downward motion, as disclosed in U.S. Pat. No. 9,199,103 B2.

The webbing of the present invention is designed for use in self-retracting lifelines that meet ANSI Standard Z359.14. Furthermore, because of the abrasion resistance and cut resistance of the outside of the webbing, the webbing is suitable for use in self-retracting lifelines having leading edge capabilities, referred to as SRL-LE devices.

Accordingly, the present invention includes a self-retracting lifeline incorporating the webbing disclosed herein, in particular, a self-retracting lifeline that meets or exceeds ANSI Standard Z359.14 and standards for self-retracting lifelines having leading edge capabilities.

Some embodiments relate to a fall-protection lanyard including the webbing described above. A fall protection lanyard is a critical component of a Personal Fall Arrest System (PFAS), used to connect the worker's body harness to an anchorage point or system. The primary purpose of a fall protection lanyard is to secure the worker at height, preventing or arresting a fall. There are several types of lanyards, each designed for specific situations and needs. For example, shock-absorbing lanyards are the most common type of fall protection lanyards. They are equipped with a built-in shock absorber which reduces the impact force on the worker's body in the event of a fall. The shock absorber does this by extending and decelerating the fall over a longer distance and time. Positioning lanyards are used to position a worker at a workstation while allowing some freedom of movement. They are not designed for fall arrest but to prevent the worker from reaching a point where they could fall. Self-retracting lanyards (SRLs) automatically extend and retract as the worker moves, allowing for some mobility. In the event of a fall, an internal braking mechanism activates, arresting the fall quickly and with minimal force on the worker. Double-legged (or twin-leg) lanyards have two legs and are used for 100% tie-off, which means the worker can remain connected to an anchor point at all times, even when moving between locations. The worker attaches one leg and then moves to the next anchor point and attaches the second leg before disconnecting the first, ensuring continuous protection. Web lanyards are made from flat, woven webbing and are often used with a shock absorber. They are lighter and more flexible than rope lanyards.

Some embodiments relate to a fall-protection anchorage including the webbing described above. A fall protection anchorage is a secure point of attachment for fall arrest equipment, such as lanyards, lifelines, and other components of a personal fall arrest system (PFAS). It's a crucial part of a fall protection system because it must be capable of supporting the forces exerted during a fall. An anchorage must be strong enough to support the weight and force of a falling person. In many regulations and standards, an anchorage is required to support at least 5,000 pounds (22.2 kN) per worker attached or must be designed, installed, and used under the supervision of a qualified person as part of a complete personal fall arrest system which maintains a

safety factor of at least two. Anchorages can vary depending on their use. They can be permanent (such as I-beams, roof trusses, or other structural members) or temporary (like portable anchorage devices that are attached to a structure).

There, of course, many alternative embodiments and modifications of the invention, which are intended to be included in the following claims.

What is claimed is:

**1. A webbing, comprising:**

- (a) a double cloth construction having (i) a first side having a plurality of warp yarns and weft yarns woven together, wherein the warp yarns are multifilament yarns comprised of ultra-high molecular weight polyethylene fibers; (ii) a second side having a plurality of warp yarns and weft yarns woven together, wherein the warp yarns are multifilament yarns comprised of ultra-high molecular weight polyethylene fibers; and (iii) a plurality of binder yarns extending between the first side and second side, whereby the binder yarns joins the first and second side together, wherein the first side of the double cloth has a face and the warp yarns of first side are predominantly exposed on the face relative to the weft yarns, and wherein the second side of the double cloth has a face and the warp yarns of the second side are predominantly exposed on the face relative to the weft yarns; and
- (b) a plurality of stuffer yarns positioned between the first side and second side of the double cloth and extending in a warp direction, wherein the stuffer yarns comprise para-aramid fibers;

wherein the webbing meets or exceeds ANSI Standard Z359.14.

**2. The webbing of claim 1, wherein the weft yarns in the first side and second side are comprised of multifilament ultra-high molecular weight polyethylene fibers.**

**3. The webbing of claim 1, wherein the first side has a first edge and a second edge and the second side has first edge and a second edge, and the weft yarns are continuously wrapped from the first side to the second side, thereby joining the (i) first edge of the first side to the first edge of the second side, and (ii) the second edge of the first side to the second edge of the second side.**

**4. The webbing of claim 1, wherein the first side and the second side are plain weaves, and a ratio of ends per inch of warp yarns comprised of UHMWPE to picks per inch in each of the first side and second side of the webbing is 3:1 or greater.**

**5. The webbing of claim 1, wherein a ratio of ends per inch of warp yarns comprised of UHMWPE to picks per inch in each of the first side and second side of the webbing is 4:1 or greater.**

**6. The webbing of claim 1, wherein three stuffer yarns are plied together to create a 3-ply yarn, and four of the 3-ply yarns are twisted together to form a cord.**

**7. The webbing of claim 1, wherein the webbing is characterized by a width, and the webbing has tensile strength of 6,000 lbs. or greater per inch of width.**

**8. The webbing of claim 1, wherein the warp yarns in the first side and second side have a denier of from 1200d to 2000d, and the first side and the second side each have from 40 to 100 warp yarns per inch.**

**9. The webbing of claim 1, wherein the weft yarns in the first side and second side have a denier of from 1200d to 2000d, and the first side and the second side each have from 6 to 18 weft yarns per inch (ppi).**

**10. The webbing of claim 1, wherein the stuffer yarns have a denier of from 800d to 2000d and a filament count of from 500 to 1500, and the stuffer yarns are provided in a range of from 100 to 250 ends per inch.**

**11. The webbing of claim 1, wherein a ratio of a combined weight of the first side and the second side to a weight of stuffer yarns ranges from 1:2 to 2:1.**

**12. The webbing of claim 1, wherein a ratio of a combined weight of the first side and the second side to a weight of stuffer yarns ranges from 1:1.5 to 1.5:1.**

**13. The webbing of claim 1, wherein the stuffer yarns consist of high-tenacity aramid fibers having a tensile strength of 2.0 GPa or greater.**

**14. The webbing of claim 1, wherein the webbing is a component of a self-retracting lifeline, a fall-protection lanyard, or a fall-protection anchorage.**

**15. A webbing, comprising:**

- (a) a double cloth construction having (i) a first side having a plurality of warp yarns and weft yarns woven together, wherein the warp yarns are multifilament yarns comprised of ultra-high molecular weight polyethylene fibers; (ii) a second side having a plurality of warp yarns and weft yarns woven together, wherein the warp yarns are multifilament yarns comprised of ultra-high molecular weight polyethylene fibers; and (iii) a plurality of binder yarns extending between the first side and second side, whereby the binder yarns joins the first and second side together; and

**(b) a plurality of stuffer yarns positioned between the first side and second side of the double cloth and extending in a warp direction, wherein the stuffer yarns comprise para-aramid fibers;**

wherein the webbing meets or exceeds ANSI Standard Z359.14.

**16. The webbing of claim 15, wherein three stuffer yarns are plied together to create a 3-ply yarn, and four of the 3-ply yarns are twisted together to form a cord.**

**17. The webbing of claim 15, wherein the stuffer yarns are selected from the group consisting of para-aramid fibers having a tensile strength of 2.0 GPa or greater.**

**18. The webbing of claim 15, wherein the stuffer yarns comprise 10 to 20 cords.**

**19. The webbing of claim 15, wherein the stuffer yarns are provided in a range of 100 to 250 yarns per inch.**

**20. The webbing of claim 15, wherein the weft yarns in the first side and second side are comprised of multifilament ultra-high molecular weight polyethylene fibers.**

**21. The webbing of claim 15, wherein the first side has a first edge and a second edge and the second side has first edge and a second edge, and the weft yarns are continuously wrapped from the first side to the second side, thereby joining the (i) first edge of the first side to the first edge of the second side, and (ii) the second edge of the first side to the second edge of the second side.**

**22. The webbing of claim 15, wherein the webbing is a component of a self-retracting lifeline, a fall-protection lanyard, or a fall-protection anchorage.**